

## UNITED STATES PATENT OFFICE

1,980,282

METHOD OF PROTECTING MAGNESIUM AND  
HIGH GRADE MAGNESIUM ALLOYS FROM  
THE ACTION OF CORRODING AGENTS

Josef Martin Michel, Bitterfeld, Germany, assignor, by mesne assignments, to Magnesium Development Corporation, a corporation of Delaware

No Drawing. Application April 1, 1931, Serial No. 527,044. In Germany April 4, 1930

4 Claims. (Cl. 148—6)

The present invention relates to a method of protecting magnesium and high grade magnesium alloys from the action of corroding agents, particularly water, alcohols, and non-oxidizable saline fluxes, at ordinary and elevated temperatures.

It has long been known that the presence of alkali chromates or chromic acid in a medium which exercises a corroding influence upon magnesium and high percentage magnesium alloys per se, causes a passivation of the metal which results in a substantial reduction or even a complete cessation of the corroding effect. It has likewise been known that a treatment of these metals with aqueous solutions containing chromic acid or alkali chromate causes the formation of a thin protective layer upon the surface of the metal or work-piece which increases its resistance to a subsequent corroding action quite generally. Simultaneously, a coloring effect is produced upon the metal surface.

I have now found that aqueous solutions of alkali sulfides cause the formation of a coherent protective layer upon magnesium and high percentage magnesium alloys. I have further discovered that exceedingly small additions of alkali sulfides when made to water, alcohols, or non-oxidizing saline fluxes and similar corroding agents, all of which are referred to in the appended claims as liquid medium, have the effect of efficiently counteracting the corroding influence of these substances. It is remarkable and of the utmost importance that the corrosive action, particularly of alcohols, is even counterbalanced at comparatively high temperatures.

Several modifications of the present invention will hereinafter be described in detail. However, I do not wish to limit the scope of my invention to such modifications, as other equally advantageous modes of applying the invention will occur to persons skilled in the art.

(1) The heat treatment of magnesium and high grade magnesium alloys at temperatures below the melting point of the metal is frequently carried out in a bath of non-oxidizing saline fluxes. The corroding action of such fluxes, which is generally but small per se, is entirely suppressed by the presence of a small quantity of alkali sulfides (sulfide of potassium, sulfide of sodium, or liver of sulfur in amounts ranging up to about 3 percent by weight of the saline flux employed).

(2) It is generally recognized that ordinary water has a slow corroding effect upon articles made of magnesium and high percentage magne-

sium alloys even at room temperatures and that this effect becomes considerably accelerated at elevated temperatures. According to the present invention an addition of about 0.2—0.5 percent of alkali sulfides is made to the water with the result that the corrosive action of the water is entirely suppressed. The small increase in weight of the articles which is frequently observed is due to the formation of a thin protective layer on the surface of the articles.

In the case of water from a water main system or from rivers, the addition of alkali sulfides causes a precipitation. It is advantageous to separate such precipitate from the water by filtering or decanting off before bringing the water into contact with magnesium or high percentage magnesium alloys, as the precipitate when settling on the surface of the metal may give rise to a pitting effect upon the latter.

(3) An increased resistance to corrosion of magnesium and high grade magnesium alloys when in contact with alcohols such as glycol, glycerine, etc., or aqueous mixtures of such alcohols, particularly at elevated temperatures, is of the utmost importance as the substances and mixtures mentioned are frequently employed as cooling liquids in internal combustion engines so as to enhance the cooling efficiency and to reduce the danger of freezing. The figures given in the following table are representative of the increased resistance to corrosion of magnesium and high percentage magnesium alloys in contact with glycol, glycerine and mixtures of both with water due to the presence of alkali sulfides. The figures given in the last column represent the corroding effect by the reduction in weight of the tested articles in grams per square meter of surface per 24 hours.

| Temperature and composition of the liquid                   | Loss in weight in grams per sq. meter per 24 hrs. |     |
|-------------------------------------------------------------|---------------------------------------------------|-----|
| Glycol 100° C.                                              | 16.6                                              | 100 |
| Glycol +0.1 percentum sulfide of potassium                  | 0                                                 |     |
| Glycol 150° C.                                              | 56.5                                              |     |
| Glycol +0.3 percentum sulfide of sodium                     | 0.10                                              |     |
| Glycerine 150° C.                                           | 9.6                                               |     |
| Glycerine +2 percentum liver of sulfur                      | 0.02                                              | 105 |
| Glycerine:water=1:1 100° C.                                 |                                                   |     |
| Glycerine:water=1:1 100° C.+0.2 percentum sulfide of sodium | 14.2                                              |     |
| Glycerine:water=1:1 100° C.                                 | 0.03                                              |     |
| Glycol:water=1:1 100° C.                                    | 6.2                                               |     |
| Glycol:water=1:1 100° C.+0.1 percentum liver of sulfur      | 0.05                                              | 110 |

(4) A permanent improvement in the resistance to corrosion of articles of magnesium and high grade magnesium alloys may be produced according to the present invention by the formation of a protective layer containing magnesium sulfide upon the surface of the articles by means of a treatment with an aqueous solution of alkali sulfides.

Sheets of a magnesium alloy are immersed in a 0.5 to 1 percent aqueous solution of sulfide of sodium at temperatures between 60 and 100° C. during a few hours. This treatment results in the formation of a protective layer containing magnesium sulfide and having a color ranging between brown and black. If sheets treated in this manner are subsequently exposed to corroding agents, for example to the action of ordinary water, a marked improvement is noticed when compared with sheets which have not been treated in this manner. The following table gives a numerical comparison of the behavior of two sheets made from the same alloy, one sheet having remained untreated whereas the other was provided with a protective surface layer by immersing it in a 0.5 percent aqueous solution of sodium sulfide at 70° C. for 10 hours. The sheets were then brought into contact with ordinary water and the amount of hydrogen developed—representing the progress of corrosion—ascertained after 24, 48 and 72 hours respectively.

I claim:—

1. A non-corrosive liquid for use in conjunction with articles consisting of magnesium and high grade magnesium alloys, characterized by the presence of a major quantity of a polyhydric alcohol and a minor quantity ranging between about 0.1 and 3 percent of an alkali sulfide in said liquid.

2. The method of protecting magnesium and magnesium alloys from the action of an alcohol-containing liquid in contact therewith, by adding to said alcohol-containing liquid alkali sulphide in amount sufficient to substantially prevent corrosion of the metal.

3. The method of counteracting the corroding influence of a polyhydric alcohol on magnesium and magnesium alloys with which said alcohol is in contact, by adding to said alcohol an amount of alkali sulphide sufficient to prevent substantial corrosion of the metal.

4. The method of counteracting the corroding influence of liquid medium upon magnesium and magnesium alloys which are in contact therewith, by adding to said medium alkali sulphide in amount sufficient to prevent substantial corrosion of the metal.

JOSEF MARTIN MICHEL.

| After hours | Development of H <sub>2</sub> in liters per sq. meter surface |                  |
|-------------|---------------------------------------------------------------|------------------|
|             | Treated sheets                                                | Untreated sheets |
| 24          | 1.5                                                           | 4.6              |
| 48          | 2.8                                                           | 7.7              |
| 72          | 4.3                                                           | 10.9             |

80

85

90

95

100

105

110

115

120

125

130

135

140

145

150